

J. H. REID.

PROCESS OF AND MATERIAL FOR REDUCING ORE AND MAKING GAS.

APPLICATION FILED JULY 16, 1920.

1,398,572.

Patented Nov. 29, 1921.



*Tested & Attest,*  
James Henry Reid,  
Bos. Hull Smith, Brook & Wm.  
*Attest.*

# UNITED STATES PATENT OFFICE.

JAMES HENRY REID, OF READSBORO, VERMONT, ASSIGNOR TO THOMAS I. HOGAN, OF BOSTON, MASSACHUSETTS.

## PROCESS OF AND MATERIAL FOR REDUCING ORE AND MAKING GAS.

1,398,572.

Specification of Letters Patent. Patented Nov. 29, 1921.

Application filed July 16, 1920. Serial No. 396,762.

To all whom it may concern:

Be it known that I, JAMES HENRY REID, a citizen of the United States, residing at Readsboro, in the county of Bennington and

5 State of Vermont, have invented a certain new and useful Improvement in Processes of and Materials for Reducing Ore and Making Gas, of which the following is a full, clear, and exact description, reference being 10 had to the accompanying drawings.

This invention relates to a process for reducing ore and for the production of gas; also to materials for realizing such processes. It is the general object of the invention to 15 reduce such ore in a more efficient manner than has been accomplished heretofore; to make it possible to utilize in the reduction of such ore (and especially of iron ore in a blast furnace) certain grades of coal the sul- 20 fur content of which has excluded them heretofore from consideration; to increase the output of the iron or other metal from blast furnaces; and to reduce the proportion of coke required for the reduction of the ore.

25 A further object of the invention is to obtain in a novel manner a large volume of gas of a heating value useful in the arts and in excess of that ordinarily obtained from the distillation of coal in retorts and in the op- 30 eration of blast furnaces. Further and more limited objects of the invention will appear hereinafter and will be realized through the steps and ingredients and the combinations thereof, respectively, embodied in the claims 35 hereto annexed. The invention will be de- 40 scribed in connection with the reduction of iron ore, for which it is especially adapted; and the drawing shows diagrammatically an apparatus or system for realizing such in- vention.

As is well known, an ordinary steel plant comprises a blast furnace, a by-product coke oven, a Bessemer converter, and an open-hearth furnace. The invention will be de- 45 scribed with reference to such ordinary steel plant equipment.

For the reduction of the iron ore and the production of gas, I first intimately mix iron ore, coking coal, and limestone ( $\text{CaCO}_3$ ) in 50 about the following proportions by weight:—

Iron ore, 100 lbs.; limestone, 42 lbs.; coal, about 80 lbs.—sufficient to produce about 60 lbs. of coke.

The limestone will first be reduced to a 55 fineness of about forty mesh, the coal to a fineness of about eight mesh, and the iron

( $\text{Fe}_2\text{O}_3$ ) will be in the finely reduced stage in which it is ordinarily supplied to blast furnaces. Where the ore is coarse or contains nodules, it is ground to a fineness of 60 about eight mesh. These ingredients, having been intimately mixed, are charged into the by-product coke oven or ovens or other retort 1 and are there retorted at a temperature of from 2600° F. to 2800° F. until 65 the coal is completely coked. By reason of the ingredients employed and the mode of treatment, all of the gases ordinarily obtained by the distillation of bituminous coal are secured; moreover, the finely divided 70 conditions of the heated mass of limestone, ore, and coal enables me to crack into gas the liquid tarry constituents of the coal, this cracking being secured by bringing the liquid tarry material into contact with a myriad 75 of incandescent bodies or points, due to the finely divided condition of the ingredients, particularly of the limestone and iron ore. As a result, the tarry constituents are removed in the retort and are recovered in the 80 form of gases which serve to enrich the gases obtained by the ordinary distillation of the coal. As the ingredients are retorted in a reducing atmosphere, at least as long as hydrocarbon vapors are present, the lime- 85 stone is not converted into lime ( $\text{CaO}$ ). The absence of tar and tarry products from the educt from the retorts greatly simplifies the recovery of ammonium sulfate from the 90 gas liquor and makes it unnecessary to pre- heat the gas or gases delivered from the retort before introducing the same into the saturator.

At the end of the retorting operation, the 95 ore will have been partly reduced by the carbon, yielding CO in accordance with the equation  $\text{Fe}_2\text{O}_3 + \text{C} = 2\text{FeO} + \text{CO}$ , this reduction being facilitated by the presence of hydrogen in the liberated gases. The ingredients will have been formed into a cemented 100 or coked mass wherein the iron ore, the carbon, and the limestone will be in most intimate contact; every small particle of ore has in close contact with it a particle of carbon and a particle of limestone, which 105 renders the mass delivered from the retorts ideal for the reduction of the ore in the blast furnace.

Among the advantages, from a gas-making standpoint, which my process, as thus 110 far described, possesses are the following:—  
(a). The recovery of a larger proportion

of gas from the coal than has been accomplished heretofore by the methods ordinarily employed, this additional recovery being due to the conversion of the tarry products into 5 gas and the production of CO through the partial reduction of the ore;

(b) The saving of heat necessary for the retorting operation, due to the conductivity of the mass therein; also due to the fact that 10 the reaction occurring within the retort is exothermic to some extent. This will result in a shorter period of time for the coking operation, offsetting largely, if not entirely, the heat required for the greater bulk 15 of material over the use of coal alone;

(c) The saving in the recovery of the by-products (such as ammonium sulfate) resulting from the gas production, due to the elimination of the tar or tarry constituents.

20 In the reduction of the ore to pig iron in the ordinary blast furnace, indicated at 2, a great saving in fuel may be accomplished by charging the said furnace with the coked or cemented mixture in a hot condition, direct 25 from the by-product oven or ovens. The saving of fuel because of this sensible heat in the charge will be enormous.

The advantage in the intimate mixture of the ingredients which enter the blast furnace 30 has already been pointed out. The flux and the reducing agent do not have to find their way around and to the ore, but are in contact with it at the very start. Furthermore, a partial reduction of the ore in the coke 35 oven has already been accomplished. This results in a quicker fusion and a quicker reduction of the ore, thus greatly increasing the output of iron from the furnace over the output secured by ordinary methods. There 40 is also a saving in the amount of coke required, since the reduction which occurs in the coke oven has been accomplished in the absence of air, and hence without the production of CO<sub>2</sub>, as is the case to some extent 45 in the blast furnace.

Reference has been made heretofore to the practicability of using coal containing a portion of sulfur which has hitherto excluded the same from consideration in connection with blast furnaces. By bringing the coke and limestone into intimate contact, so that every small particle of coke has next to it a similar particle of limestone, the sulfur in the coke will be absorbed by the 50 lime and will not enter the iron. While it is true that iron at a white heat will absorb sulfur from calcium sulfate, in the reducing atmosphere of the furnace calcium sulfate will not be formed, but rather calcium sulfide, and the sulfur constituent of the coal will be absorbed by the calcium constituent 55 of the limestone.

In the operation of the blast furnace, the ore will not only be quickly reduced, with 60 the advantages hereinbefore described, but

a large volume of carbon monoxide will be produced which may be mixed with the gases formed in and discharged from the coke oven; and the resultant mixture of these gases may be used for the open hearth furnace and for various commercial purposes. 70

In the drawing, the gas from the retort (or by-product coke oven or ovens) 1 and from the blast furnace 2 are conducted by the pipes 3 and 4 to a hydraulic main 5, as 75 well as through the usual purifiers and scrubbers (not shown), being finally delivered to a gas holder 6. From this holder, such proportion of the gas as may be desirable may be supplied to an open hearth furnace or furnaces 7 by a pipe or pipes 8.

From a charge of about 80 lbs. of coal, 100 lbs. iron ore, and 42 lbs. limestone, there will be recovered in the coke oven about 600 cu. ft. of 500 B. T. U. gas, or a total of 80 300,000 B. T. U. In addition, the reduction of the Fe<sub>2</sub>O<sub>3</sub> to FeO will yield about 182 cu. ft. of 323 B. T. U. gas, or a total of 58,786 B. T. U., making a total B. T. U. recovery from the 80 lbs. of coal in the coke 90 oven of 358,786 B. T. U.

In the blast furnace, the ore, coke, and limestone will yield approximately 5000 cu. ft. of gas with a total B. T. U. value of 475,000. The total B. T. U. recovery from 95 the 80 lbs. of coal first introduced into the coke oven will amount to 833,000, or 10,400 B. T. U. per pound of coal. The recovery of useful gas by the process herein described represents more than 70 per cent. of the 100 potential energy of the coal employed in the process. The limestone serves as a gas activating agent in the retort and as a fluxing agent and a gas-activating agent in the furnace. 105

Having thus described my invention, what I claim is:

1. The process which comprises retorting a mixture of ore with cokable carbonaceous material and material capable of acting as 110 a fluxing agent and of activating the evolution of gas, thereby to produce a coked aggregate without material conversion or alteration of the said agent, and smelting the said aggregate. 115

2. The process which comprises coking a mixture of ore, cokable coal and a fluxing and gas-activating agent, without substantial alteration or conversion of said agent, and treating the coked aggregate, thus produced, in a blast furnace. 120

3. The process which comprises coking a mixture of ore, cokable coal, and limestone, without substantial conversion or alteration of the limestone, whereby the limestone may 125 serve as a gaseous activating agent and as a fluxing agent, and smelting the coked aggregate.

4. The process which comprises coking a mixture of approximately 100 parts by 130

weight of ore to 40 parts by weight of limestone to 80 parts by weight of bituminous coal, and without substantial conversion or reduction of the limestone, whereby the limestone may serve as a gas-activating agent and a fluxing agent, and smelting the resultant aggregate.

5. The process of reducing ore which comprises smelting a coked mixture of ore and 10 carbonaceous material with limestone, the limestone being present in proportion to constitute a fluxing agent and a gas-activating agent.

6. The process of reducing ore which comprises treating in a blast furnace a coked mixture of iron ore, carbonaceous material and limestone in about the following proportions by weight: 100 parts ore, 60 parts coke, 40 parts limestone, whereby the limestone is capable of acting as a fluxing agent and a gas-activating agent.

7. The process of reducing ore which comprises treating in a blast furnace a coked

mixture of ore, carbonaceous material, and a fluxing and gas-activating agent.

8. Material for the reduction of ore and the production of gas comprising a coked mixture of ore, carbonaceous material, and a fluxing and gas-activating agent.

9. Material for the reduction of ore and 30 the production of gas comprising a coked mixture of iron ore and carbon with limestone, the limestone being present in proportion to constitute a fluxing and a gas-activating agent.

10. Material for the reduction of ore and the production of gas comprising a coked mixture of iron ore, carbon and limestone in about the proportions by weight of 100 parts ore, 60 parts carbon and 40 parts limestone, 40 whereby the limestone may serve both as a fluxing agent and a gas-activating agent.

In testimony whereof, I hereunto affix my signature.

JAMES HENRY REID.